

Aug. 31, 1943.

H. A. DOERNER

2,328,202

PROCESS FOR PRODUCING MAGNESIUM METAL

Filed Dec. 30, 1940

5 Sheets-Sheet 1



Aug. 31, 1943.

H. A. DOERNER

2,328,202

PROCESS FOR PRODUCING MAGNESIUM METAL

Filed Dec. 30, 1940

5 Sheets-Sheet 2



Aug. 31, 1943.

H. A. DOERNER

**2,328,202**

## PROCESS FOR PRODUCING MAGNESIUM METAL

Filed Dec. 30, 1940

5 Sheets-Sheet 3



INVENTOR  
HENRY A. DOERNER  
BY *O.W. Lee*  
ATTORNEY

Aug. 31, 1943.

H. A. DOERNER

2,328,202

PROCESS FOR PRODUCING MAGNESIUM METAL

Filed Dec. 30, 1940

5 Sheets-Sheet 4

FIG. 4



Aug. 31, 1943.

H. A. DOERNER

2,328,202

PROCESS FOR PRODUCING MAGNESIUM METAL.

Filed Dec. 30, 1940

5 Sheets-Sheet 5



FIG. 5



FIG. 7



FIG. 6

INVENTOR  
HENRY A. DOERNER  
BY *O.W. Lee*  
ATTORNEY

## UNITED STATES PATENT OFFICE

2,328,202

## PROCESS FOR PRODUCING MAGNESIUM METAL

Henry A. Doerner, Pullman, Wash.

Application December 30, 1940, Serial No. 372,293

19 Claims. (Cl. 75—67)

The present invention relates to an improved process for producing magnesium metal and involves the electrothermal reduction of magnesium oxide by carbon, and the subsequent steps to obtain the magnesium metal in solid mass form of high purity.

According to my invention a mixture of carbon and magnesium oxide is reduced to magnesium vapor and carbon monoxide in a thermal reduction furnace at a temperature of approximately 2000° C. preferably by means of an electric arc. The magnesium vapor and carbon monoxide issue as a blast from the reduction furnace directly into a cooling flue into which is atomized a controlled quantity of a readily volatile inert liquid containing a suitable proportion of hydrocarbon oil having a boiling point above the constant temperature of the cooling fluid which is maintained at about 200° C. principally by the negative latent heat of vaporization of the volatile liquid supplied. Thus the magnesium vapor is immediately shock cooled to well below the melting point of the metal so as to substantially prevent the reoxidation which would otherwise occur in the presence of the inherently existing carbon monoxide. The magnesium condenses in almost atomic particles and is entrapped by the atomized hydrocarbon oil which serves as a vehicle to carry the magnesium and other inherently existing solids through a suitable separator where the vaporized portions of the cooling liquid and carbon monoxide are discharged into a suitable condenser, and the magnesium laden oil is removed to a retort and the oil distilled off at a temperature below the melting point of magnesium and in an inert atmosphere, as for instance, the vapors and gases produced by the distillation of the hydrocarbon oil will suffice for the requirements when air is excluded.

Distilling off the hydrocarbon oil, provides a porous mass of the existing solids throughout which is a dispersion of pyrophoric magnesium and a small amount of the hydrocarbon oil which fails to distill off. Preferably, this oil distillation is conducted in molds so as to form molded briquettes and thus lessen the possibility of dust contamination during the subsequent distillation of the magnesium.

These porous briquettes containing the finely divided magnesium are then discharged into another retort, and the magnesium is distilled, preferably at a temperature slightly below its boiling point, say 1000° C. and the metal is promptly condensed, preferably at a temperature slightly above the melting point; the dis-

tilling and condensing being done in an inert atmosphere. The molten metal can then be drawn off and cast in any suitable solid form. Preferably, the distilling of the magnesium is conducted in a continuous series of separate charges, and the exhausted briquettes are serially discharged to make way for recharging.

In the thermal reduction of magnesium oxide with carbon, the reaction occurs in accordance with the equation:



and since the thermal reduction temperature is far above the boiling point of magnesium, the metal is produced in the vapor form. In actual practice, the reduction products are always intermingled with some finely divided solids. These solids are mainly MgO and C and are due to particles of the original charge which are carried out of the reduction furnace without reacting, and also due to partial reversal of the reaction, occurring at the outlet of the reduction furnace, together with such impurities as may exist. These solids in fine powder, are intermingled with the Mg vapor and CO, and it is utterly impossible to obtain isolated Mg by shock cooling of the reaction products.

Any form of shock cooling will condense the Mg in almost atomic particles intermingled with the other finely divided solids, and the Mg can not be successfully recovered by distillation unless some form of bonding is employed, so as to obviate dust being carried over with the metal vapor.

If the Mg is shock cooled by a liquid essentially non-volatile at the cooling temperature, there will be such an extreme excess of the cooling liquid that it will be exceedingly difficult and expensive to separate the excess of liquid so as to proceed further with recovering the Mg by distillation.

To form the finely divided Mg and other solids into a fluid paste which can be satisfactorily processed, there is required about two pounds of hydrocarbon oil to each pound of total solids collected therein, the ratio depending upon the existing proportion of non-metallic contents. There is no known hydrocarbon oil which will produce the required temperature reduction when atomized into the thermal reduction products at such a minor rate. In fact it would require more than sixty times that amount of hydrocarbon oil when substantially non-volatile at a satisfactory cooling temperature, and the same would be true of any other liquid hydrocarbon

substantially non-volatile at the cooling temperature employed. It is commercially prohibitive to attempt to separate such an extreme excess of liquid by centrifuge, or otherwise.

For these reasons, the present invention accomplishes the shock cooling by the vaporization of a hydrocarbon liquid sprayed into the reaction products at a controlled rate to produce a cooling temperature which will provide a dew point at which the unvaporized portion of the hydrocarbon liquid will be about twice the weight of the total solids collected therein.

Various cooling liquids may be employed, provided that they are chemically inert to the existing conditions. Liquid hydrocarbons are particularly suited for the purpose, provided that their boiling point range is within the limits which will afford an adequate cooling temperature at which the unvaporized portion can be controlled to meet the previously stated requirements. Preferably, the unvaporized portion should contain sufficient carbonizing oil to later afford satisfactory bonding of the solids collected by the shock cooling, because otherwise there will be considerable dusting which makes difficulty in recovering the Mg by distillation.

To illustrate one example, one part of lubricating oil S. A. E. 30 and sixteen parts of gasoline will suffice for the required purpose. This mixture is sprayed into the reduction products at a controlled rate in accordance with the output of the reduction furnace, so as to produce a cooling temperature of say 190° C. This will vaporize practically all of the gasoline and practically none of the lubricating oil, and there will be about two pounds of oil to each pound of Mg and other solids collected therein, and if this proves to be more oil than is required, the rate of spray can be reduced so as to supply less oil, and also the temperature will rise in accordance with the decrease in the amount of gasoline supplied for vaporization. Conversely, if more oil is required for proper fluidity, the rate of spray can be increased to supply more oil, and in this instance the temperature will decrease in accordance with the increase in the amount of gasoline supplied for vaporization. If necessary, the rate of spray can be increased until the temperature is decreased sufficiently to afford a dew point for the heavier fractions of gasoline and thereby cause a portion of them to condense. However, such a situation is merely illustrative and need never occur, it is mentioned for the purpose of illustrating the possibility of condensing different fractions of the cooling liquid. As for instance, instead of the described gasoline and oil mixture, there may be used some low priced hydrocarbon liquid having several constituents and a boiling point range suited for the purpose. As for instance, the commercially obtainable stove oil will suffice, provided that it is sprayed at a controlled rate to produce a cooling temperature which will afford a dew point at which the unvaporized portion is the correct amount for collecting the Mg and other solids. With such a cooling liquid, each change in the cooling temperature will alter the amount of heavier fractions vaporized, because the boiling points of these various fractions are much closer together than was the case in the previous mixture of gasoline and oil, and therefore each temperature drop will afford a dew point for an additional fraction.

The stove oil is sprayed into the thermal reduction products at a controlled rate to produce a cooling temperature of say 185° C. to afford a

dew point at which the unvaporized heavier fractions will be about two pounds to each pound of Mg and other solids collected therein. Then each increase in the rate of spray will reduce the temperature and increase the percentage of unvaporized constituents, so that each increase in the rate of spray will have an accumulative effect on the percentage of unvaporized constituents. Thus the unvaporized portion used for collecting the Mg and other solids can be varied considerably with but slight changes in the cooling temperature.

In this manner the spray rate can be set at whatever volume will produce a temperature which will afford the proper amount of unvaporized liquid for properly carrying out the process, and the ratio of unvaporized liquid can be repeatedly altered according to requirements, with but minor changes in the cooling temperature. The control can readily be made automatic by a thermostat, and reset as often as occasion requires, to meet existing conditions.

This improved method affords the advantage that the shock cooling is accomplished by vaporizing about 94 percent of the cooling liquid, thereby affording collection of the Mg and other solids in about 6 percent of the total cooling liquid employed, so as to form a fluid paste which can be quickly separated from the CO and hydrocarbon vapors, so that the latter can be condensed to liquid for repeated use. The fluid paste is conducted away as fast as it is formed, and is in condition for immediate briquetting, without resorting to such procedures as centrifuging or filtering to reduce the quantity of liquid. The hydrocarbon oil is distilled off during the briquetting and condensed to liquid for repeated use. The briquetting proceeds at the same rate as the output from the reduction furnace, and then the distilling of the Mg follows in immediate sequence and at the same rate.

Thus the shock cooling, collecting, separation, bonding, and distilling, are united into a continuous process which is accomplished in a regular sequence of steps without interruption, and where each step is correlated with the other steps.

During the briquetting and distilling of the Mg, there occurs some thermal decomposition of the hydrocarbons which results in the formation of gases such as hydrogen and methane and these gases are utilized to afford an inert atmosphere during the briquetting and distilling, after which the gases are collected as a by-product. Thermal decomposition of hydrocarbons at the cooling zone also produces some hydrogen and methane intermingled with the existing CO and these gases are collected as a by-product having considerable fuel value.

The present process has been discovered and perfected by extensive experiments and experience, by actually operating the process and successfully producing magnesium metal in solid cast form with a high state of purity and a bright lustre.

The accompanying drawings illustrate the best mode that I have thus far devised for carrying the process of my invention into actual practice. A consideration of these drawings in connection with the following specification relating thereto, will afford a full understanding of the various details relating to the coordinating of the cooling temperature with the quantity and quality of liquid employed, and with relation to the output of the thermal reduction furnace, so as to assure efficient operation in the necessary intervals.

of separation, briquetting, distillation and condensing of the magnesium; together with the procedures for recovering and repeatedly utilizing the hydrocarbon oil and the volatile liquid employed for cooling; and the utilization of the permanent gases as a part of the process.

Fig. 1 diagrammatically shows the general organization of equipment suitable for accomplishing the process.

Fig. 2 is a vertical section of the major portion of the equipment.

Fig. 3 is a vertical section of the two retorts with part of the heat insulating material removed to disclose the condenser.

Fig. 4 is a vertical transverse section taken on the line 4—4 of Fig. 3 and enlarged to represent proportionate size relative to the showing in Fig. 2.

Fig. 5 is an enlarged horizontal section taken on the line 5—5 of Fig. 2.

Fig. 6 is a perspective view of one of the multiple briquette molds carried on paired sprocket chains.

Fig. 7 is a perspective view of one of the series of cages from which the magnesium is distilled.

First referring to the illustrated equipment broadly, there is shown a thermal reduction furnace E provided with an automatic feed mechanism collectively indicated at D, and supplied with material from the hopper B. The thermal reduction takes place in this furnace E and the reduction products issue as a blast through the flue F where they are shock cooled by the vaporization of the major portion of a spray of liquid hydrocarbons fed through the pipe 28, and the unvaporized hydrocarbons entrap the Mg and other solids and this mixture issues as a fine mist into the separator G from which the mixture is promptly discharged as a fluid paste into the vertical pipe H and conveyed to the heated retort L where the hydrocarbons are distilled off and the Mg and other solids formed into briquettes which are then fed into the heated retort M where the Mg is distilled off and then condensed as a highly pure metal.

The scrubber S, reservoir R, and condensers C—C' afford means for recovering the vaporized hydrocarbons for repeated use, and the tank T supplies the reservoir R to replenish the hydrocarbons consumed in the process. The exit gases may be metered as indicated at N.

The process is carried out by coordination of the various steps, so as to assure efficient operation in regular sequence, without interruption and delay. The preferred mode of accomplishing each step will now be described in detail.

#### Thermal reduction

The thermal reduction furnace may be of any suitable type, and the charge of MgO and C may be fed thereto in any suitable manner, either dry or admixed with a liquid hydrocarbon. As shown in Fig. 2 the reduction furnace E consists of a refractory muffle 24 surrounded by loose packed refractory, suitably water jacketed as indicated at 23 and sealed by a water jacketed cover 21 at 23 and sealed by a water jacketed cover 21 electrically insulated as indicated at 22. The electrode 16 passes through the insulated cover 21 and is automatically advanced by a carriage mechanism which is collectively indicated at A and actuated by a worm reduction unit 20 turned by the motor 19 which is driven in accordance with the potential across the arc in the reduction furnace. Suitable power source is connected to the sliding friction terminal 18 which is freely

movable along the electrode 16 so as to accommodate the advancement thereof and the feeding in of a new electrode 16' without interrupting the current. The insulated clamp 17 is provided for convenience in affording a new bite on the electrode each time the carriage is raised from its lowermost position to start another descent.

The electrode 26 is secured to the frame of the reduction furnace and connected to the source of power. This electrode 26 is hollow and provides the feed port for the reduction furnace. In the present instance, there is collectively indicated at D, a hydraulic feed mechanism which is automatically operated by electromagnetic valves. The charge from the hopper B is packed in metal cartridges such as 27 and 27' which have both ends open. An electric vibrator 10 is used to tightly pack the dry powdered material in the cartridges which are arranged in an endless train and passed along a track from the packing position to the feed port of the reduction furnace and back again on a return track by opposite movements of the reciprocating carriages 2 and 3 supplemented by the necessary cross movements which are accomplished by levers (not shown) mechanically actuated by the movement of these carriages which are operated by the hydraulic rams 8 and 9.

The carriages 2 and 3 are slidably mounted in guideways and each of these carriages consists of two separately movable sections which fit around each carriage, and the outward movement of each carriage separates its two sections to provide for inserting and removing the cartridges. These two carriages alternately move outwardly from their illustrated positions, to close the respective ports in the hopper and in the reduction furnace, after which the cross movement of the respective cartridges is accomplished and each carriage alternately returned to their illustrated positions to register an empty cartridge under the hopper and a filled cartridge under the feed port of the reduction furnace where the charge is very gradually injected into the furnace by the ram 4.

The rams 8, 9, and 4 are supplied with pressure through the electromagnetic valves 11, 12, 13 and 14, the first three of which are suitably connected to an air pressure line and the last to oil under pressure from the pump P for which it forms a by-pass in the manner illustrated. The rams 8 and 9 are each provided with an oil reservoir such as 0 which is subject to the air pressure from their respective valves, each of which has a discharge line for conducting any oil froth to a suitable reservoir not shown. One side of each ram is operated by air pressure and the opposite side by oil under air pressure. This provides a more even control than would otherwise be afforded by air pressure alone.

The injecting ram 4 is attached to the carriage 3 and connected to its pressure lines by flexible tubing so as to accommodate its movement with the carriage 3.

The various movements of the rams operate electrical switches which control the magnetic valves either directly or else through a relay 15. The circuits are so arranged that when the filled cartridge 27 is registered in position under the feed port as illustrated, a switch is operated to cause the electromagnetic valve 14 to close the by-pass so as to supply hydraulic pressure from the pump P to very gradually raise the injecting ram 4 so that its plunger 5 will gradually push the charge out of the cartridge and into the feed port 75 of the reduction furnace. The completed stroke

operates a switch which causes the magnetic valve 14 to open the by-pass and leave the ram 4 at its ascended position; and this same switch also operates the magnetic valve 13 to actuate the ram 9 so that the carriage 3 and ram 4 carried thereby are moved to the right until the upper plate of this carriage closes the feed port of the reduction furnace, whereupon the carriage is halted by a mechanical stop, and an electrical switch operates the magnetic valve 11 to quickly lower the ram 4 which then operates a switch to cause the magnetic trigger 7 to release the toggle lever 6, whereupon the ram 9 completes its outward stroke and this movement separates the reciprocating sections of the carriage and also mechanically actuates a lever (not shown) which moves a full cartridge into position and removes the empty as the ram reaches the end of its movement, whereupon a switch operates the magnetic valve 13 to reverse the ram 9 which moves the sections of the carriage 3 together and carries the filled cartridge and the ram 4 to the left and again in register with the feed port of the reduction furnace, whereupon the first mentioned switch is again operated to cause the magnetic valve 14 to close the by-pass so as to again raise the ram 4 to begin another cycle. This movement of the carriage 3 to the left also moves the train of empty cartridges towards the hopper.

The two sections of the carriage 2 are latched together and their movement begins when the carriage 3 reaches its illustrated position, at which time the switch which closes the by-pass valve 14, also operates the magnetic valve 12 to actuate the ram 8 to move the carriage 2 to the left and close the port in the hopper. This movement unlatches the sections and the outer section continues its movement to separate the sections and mechanically actuate a lever (not shown) to move an empty cartridge into place and push out the filled cartridge into the line of travel. The full movement of this carriage operates a switch which causes the magnetic valve 12 to reverse the ram 8 and move the carriage 2 back to its illustrated position thereby moving the train of filled cartridges towards the reduction furnace and the empty cartridge in register with the open port of the hopper where it is subjected to the action of the electric vibrator 10 until the beginning of the next rising stroke of the ram 4. This vibration assures that each cartridge will be tightly packed with the material from the hopper, thus substantially eliminating the possibility of inclusions of air, and also assuring a compact charge which can be effectively injected by the plunger 5 of the injecting ram 4. The feed port of the reduction furnace is of sufficient length to contain four or five of these tightly packed charges and thus there is provided an effective air seal for the reduction furnace. The pump P can be driven by a variable speed motor controlled by a suitable rheostat and the rate of feed to the furnace can readily be regulated according to the best operating conditions.

This automatic feed device is preferable because it provides exceptional uniformity of the operation of the thermal reduction furnace and prevents fluctuations in the output of the thermal reduction products. However, any suitable form of feed device may be substituted for the disclosed embodiment, which is hereby acknowledged to be the sole invention of Elmer Donald Dilling and is separately disclosed and claimed in his application Serial No. 473,323 filed January 23, 1943.

#### Shock cooling and separation

The cooling flue F is mounted at the outlet orifice d of the reduction furnace and securely held in fixed relation thereto. As shown in Fig. 5 this flue F is water jacketed and its inner end is provided with a spray ring which may have either one or two annular spray channels such as U and V each provided with a multiplicity of spray orifices opening into the flue F. In the present instance the spray channel V is shown connected to the pipe 28 which supplies liquid hydrocarbons under pressure from the reservoir R, a pump such as 30 providing the necessary pressure, and any suitable means may be provided to control the flow through the pipe 28, as for instance the hand operated valve 29 will suffice.

The thermal reduction products consisting of Mg vapor and CO, together with some MgO and C, issue as a blast from the reduction furnace E into the flue F where they contact the multiplicity of streams of liquid hydrocarbons issuing from the orifices of the spray channel. This blast is sufficient to substantially atomize the liquid hydrocarbons, and complete vaporization thereof will take place until the supply through the pipe 28 is sufficient to reduce the temperature sufficiently to afford a dew point for the heavier fractions of the liquid hydrocarbons supplied, as for instance stove oil. The flow through the pipe 28 is regulated so that a suitable percentage of the liquid is unvaporized, say about 5 per cent. The vaporized portions effectively reduce the temperature of the thermal reduction products, and the negative heat of vaporization of the sprayed liquid greatly reduces the amount of liquid required. This leaves the unvaporized portion disseminated and its effectively entraps the condensed Mg and other solids, and this mixture passes into the separator G as a mist which is forced out into the vertical pipe H as a fluid paste, and the CO and vaporized hydrocarbons pass out through the pipe 49 to the scrubber S. Any suitable separator may be employed, but in the present instance the separator G is shown as a closed vertical casing, heat insulated and having a vertical slot 43 opening into the vertical pipe H. Rotatably mounted within this casing is a vertical shaft 38 having a number of spiders such as 39 which support four blades such as 40. This shaft and its blades are motor driven as indicated at 45 and are turned at sufficient rate to urge the before mentioned mist to the walls of the casing and carry the coalescing globules around the casing until they escape through the open slot 43 into the vertical pipe H in the form of a fluid paste. This shaft 38 is driven at sufficient speed that the movement of the blades precludes any of the mist forming a liquid in the bottom of the casing, where the shaft 38 is further provided with a spider 44 which would urge any such condensate out through the lower part of the slot 43 and prevent accumulation in the separator.

The vaporized hydrocarbons and existing gases must of necessity rise in the separator, and pass out through the pipe 49 into the scrubber S. To assure complete separation of the mist from the vaporized hydrocarbons and gases, the spiders 39 are provided with disks 41 and rings 42 alternately arranged on the several spiders to serve as baffles to produce a zig-zag path through the separator G.

75 Mounted in the upper part of the separator G

is a thermocouple 37 which senses the existing temperature in the separator, so as to provide for automatic control of the rate of liquid flow through the pipe 28 to maintain a constant temperature and uniform relation with the output of the thermal reduction furnace.

This thermocouple is shown connected to the potentiometer 34 through which the motor 35 is turned so as to vary the rheostat 36 which controls the speed of the variable speed motor 31 which drives the pump 30 supplying the hydrocarbon liquid to the flue F through the pipe 28.

By providing the reservoir R with a hydrocarbon liquid which will readily vaporize in the flue F to produce a suitable cooling temperature of say about 200° C. and leave an unvaporized portion sufficient to form a fluid paste with the finely divided Mg and other solids, the ratio of the vaporized and unvaporized portions can readily be controlled by altering the rate of flow through the pipe 28, either by automatic control to maintain a constant temperature in the separator G or else by manually regulating the valve 29 in the pipe 28, or by manually operating a suitable rheostat to control the speed of the motor 31. In any instance the requirements will be determined by an inspection of the fluid paste formed and careful judgment of the efficiency of the existing operation, then the conditions can be appropriately altered as circumstances may suggest and necessity require. That is to say, that a deficiency in the collecting liquid may be corrected either by reconditioning the liquid in the reservoir R, or else by altering the cooling temperature and rate of spray according to requirements and according to the character of the liquid supplied from the reservoir R. Successful operation permits of reasonable latitude and there is no necessity for frequent changes from a properly established ratio.

As was hereinbefore mentioned, there is always present in the output of the reduction furnace, some MgO and carbon due to reversal of the reaction at the outlet orifice of the reduction furnace and usually some impurities such as silicon and its compounds. Such solids are inclined to form a hard deposit in the outlet orifice and block the output of the reduction furnace. To take care of this unavoidable condition, I prefer to provide an automatic reamer as collectively indicated at Z in Fig. 5. This reamer is driven by a motor, and a ram supplements the rotary movement by a reciprocating action which periodically enters this rotating reamer into the outlet orifice of the reduction furnace and promptly withdraws it so as not to appreciably impede the output from the furnace. As here shown, this reamer passes tangentially through the separator G and axially enters the flue F which is correspondingly positioned for this purpose.

As shown in Fig. 5, this rotary and reciprocating action is accomplished by providing a hydraulic cylinder 64 with a piston 66 having a sleeve 65 extending full length of the cylinder 64 and slidably mounted through the forward head 68 of the cylinder. A tubular bearing 69 having a flange 76 is rotatably mounted in the sleeve 65 and held by a nut 70. The motor 72 has an elongated shaft 67 which passes through the cylinder head 71 and is slidably keyed to the tubular bearing 69 in such manner as to accommodate full movement of the piston 66. Secured to the outer end 76 of the tubular bearing 69 is a bit 75 having a reamer head 73 and carry-

ing a pair of small propellers 74. From this description it will be seen that the bit 75 rotates with the shaft 67 and is reciprocated by the movements of the piston 66.

Pressure is alternately applied to opposite sides of the piston 66 through the pipes 77 and 78 by any suitable control such as a magnetic valve periodically operated, as for instance by a clock switch, so that the reamer head 73 periodically enters the outlet orifice of the reduction furnace and is promptly withdrawn, the propellers 74 sufficing to remove any solids from the flue F.

When properly collected, the before mentioned MgO and C afford a very desirable bulking agent for briquetting the Mg, and for this purpose the unvaporized portion of the hydrocarbon liquid should contain sufficient oil of a character to afford a suitable bonding agent when carbonized at a temperature below the melting point of Mg. However, if it is desired to resort to separately adding a bonding agent, the unvaporized collecting liquid may be of the same character as the vaporized portion by supplying the reservoir R with a light hydrocarbon and controlling the rate of flow through the pipe 28 to produce a cooling temperature which will produce a dew point so as to preclude total vaporization. No advantage is seen in resorting to this variation and it is mentioned merely as a possible alternative.

#### Conveying

The vertical pipe H is connected to the pump 47 driven by the motor 48, and the fluid paste containing the Mg, MgO, C and any solid impurities, all suspended in hydrocarbon oil, is conveyed by the pipe 46 direct to a hopper 80 above the briquetting retort L where it is fed into this retort by a motor driven pump as indicated at 81 in Fig. 3. Here it should be noted that the fluid paste is conveyed directly from the separator G to the briquetting retort L without resorting to filtering nor centrifuging, either of which are highly impractical because the Mg is inherently in almost atomic particles, and it is therefore difficult and expensive to separate any excess of oil which would otherwise exist in the absence of the present processes which is particularly directed to avoiding that commercially impractical inaptitude.

#### Briquetting

As shown in Fig. 3 the briquetting retort L consists of a horizontal tube 82 rectangular in cross section and heated by electrical resistance elements as indicated at 83, and suitably heat insulated. Passing through this retort, is an endless conveyor having paired chains such as 86 which are trained around paired sprocket wheels such as 84 and motor driven at the opposite end 60 by paired sprocket wheels such as 87. Pivoted to these sprocket chains is a series of overlapping pans 85 each of which is formed with a number of basins such as Y for carrying the fluid paste through the retort so as to form briquettes molded to the shape of these basins. During the movement of each pan 85 around the drive wheels 87, the pan swings on its pivots to an inverted position where its swinging movement is abruptly halted by striking the bumper 88, whereupon the briquettes drop into the hopper 89. The return flight of the conveyor passes through the rectangular tube 91 which is provided with an expansion joint as indicated at 92. The entire mechanism is enclosed air tight.

From the hopper 80 the fluid paste is continu-

ously fed into the molding pans 85 by the motor driven pump 81 having a number of outlet nipples as indicated at K in Fig. 4 corresponding to the number of basins in each of the pans 85 which are shown in Fig. 6 as each having four basins. The pans being overlapping as shown, their travel and the feed from the pump 81 can both be continuous, and the fluid paste will readily find its level in the basins of each separate pan, so as to form molded briquettes when the oil is distilled off.

The retort tube 82 is maintained at a suitable temperature of say about 500° C.; and as the pans 85 pass through the retort, the oil is distilled off and portions thereof are carbonized to afford a bonding agent for the briquettes. This heating forms some hydrogen and methane by thermal decomposition of the hydrocarbon oil, and these gases and the vaporized oil pass out through a pipe 93 into a condenser C' and this directional flow is assisted by recirculating these gases into the opposite end of the retort through a pipe 95 from the motor driven pump 96 which is fed by the pipe 94 from the condenser C', thus forming a continuous circuit for the repeated utilization of the same gases which are derived from the process itself. The retort being originally supplied with a suitable gas such as methane or else hydrogen, any losses will be fully replenished by thermal decomposition of a part of the hydrocarbon oil during the briquetting, and any excess of such gases will pass through the pipe 133 into the meter N' and out through the pipe 135 to the pump 33 of Fig. 2. The liquid condensate from the condenser C' is constantly returned to the reservoir R through the pipes 61' and 61.

#### *Magnesium distillation*

The molded briquettes are porous cakes of the existing solids throughout which is a dispersion of pyrophoric Mg and a small amount of hydrocarbon oil. These briquettes are preferably about the length of a finger and of sufficient thickness to not be very fragile. The Mg can readily be distilled from these porous briquettes without the occurrence of any bleeding of liquid Mg from the briquettes, because the Mg is so finely distributed throughout the porous mass that vaporization occurs without appreciable coalescing during the liquid state.

The Mg can be distilled from these briquettes in any suitable manner; however, it is preferable to avoid any procedure which causes crushing and attrition, so as to minimize the amount of dust carried over by the Mg vapors.

As shown in Fig. 3 the Mg distilling retort M is connected direct to the briquetting retort L by the hoppers 89 and 97 which are provided with the bell gate 90. This retort M consists of a horizontal tube 98 rectangular in cross section and heated by electrical resistance elements as indicated at 100. The adit end of the rectangular retort tube 98 is connected by an expansion joint 99 to the upper part of a housing 101 which has its lower part connected to a horizontal casing 102, and the opposite end of this casing is connected to the discharge end of the retort tube by means of a curved tube 103 of slightly larger rectangular cross section than the retort tube. The entire assembly is air tight and suitably heat insulated.

Due to the fact that this retort is heated to 1000° C. it is impractical to pass a conveyor through the retort, and therefore the present invention provides a novel means to continuously

5 pass the briquettes through the retort. The retort tube 98 is filled with a line of cages such as 104 which have large openings 105 in their ends for the passage of gas through the briquettes during distillation. These cages are passed through the retort by a periodically operated hydraulic ram 108, which is mounted on the housing 101 and in line with the retort tube 98. The cages pass around the curved tube 103 and arrive in an inverted position on a pair of tracks 109 over the hopper 110 into which the exhausted briquettes are discharged. The bell gate 126 is used to drop the exhausted briquettes into the hopper 127 from which they may be removed in any suitable manner, one form of which is shown at 128.

15 These exhausted briquettes contain principally MgO and C, and since these constituents are the same as the original reactants, it is feasible to subject this discharged material to the described process and gain the Mg therefrom, to thereby enhance the percentage of recovery. Of course such reprocessing requires adding sufficient MgO to afford a proper ratio for thermal reduction. It is also feasible to first grind these exhausted briquettes and subject the material to flotation to separate any silicates or other impurities so that the reprocessing by thermal reduction will not result in an accumulated percentage of impurities.

30 The cages 104 are individually returned to the adit end of the retort tube 98 by means of an endless conveyor operating in the casing 102 and housing 101. This conveyor consists of a pair of sprocket chains such as 111 trained around a pair of wheels such as 112 spaced apart on opposite sides of the paired tracks 109, and these sprocket chains then pass through the horizontal casing 102 and are trained around a pair of drive wheels such as 113 and then under idler wheels such as 114 and back through the casing to the wheels 112. These sprocket chains are connected by one or more cross bars such as 115 which serve to drag each inverted cage through the casing and into the housing 101 where the curved track 116 supports each cage until it arrives in upright position at the adit end of the retort. The cross bar 115 then passes on and moves a lever 117 which makes an electrical contact which 35 operates a magnetic valve 118 to actuate the hydraulic ram 108 to cause its plunger 119 to move the line of cages exactly one cage length. When the cross bar 115 leaves the lever 117 the magnetic valve 118 reverses the ram and retracts 40 its plunger out of the path of travel, where it remains until the next movement of the lever.

45 As seen in Fig. 3, the second cage in line is positioned under the hopper 97, and the briquettes drop into the cage by gravity, and any stray briquettes will be caught by the empty cage already in position. The bell gate 90 is used to keep the hopper 97 supplied with sufficient briquettes to completely fill each cage 104 so that the retort tube 98 is at all times completely filled 50 with briquettes. This bell gate 90 is here shown as operated by a hand lever but it may very well be automatically operated either hydraulically or mechanically.

55 At the center of the retort 98 is a tube 122 which conducts the vapors to a heated dust separator 123 in the manner best seen in Fig. 4, a suction clean-out tube being indicated at 124. The outlet neck 125 of this dust collector connects to the condenser W.

The briquettes contain some hydrocarbon oil,

and the temperature of the retort M is sufficient to thermally decompose substantially all of this oil into gases, principally hydrogen and methane. To accelerate the distillation of the Mg and maintain a directional flow of the vapors, each end of the retort tube is supplied with gas through the pipes 120 and 121 from the pump 96. This gas passes through the openings 105 in the ends of the cages and through the porous briquettes to greatly assist in removing the Mg in vapor form. To assist in this directional flow the bell gate 90 is provided to separate the retort M from the retort L and thus prevent inter-circulation between the two retorts.

#### Condensing

Any suitable condenser may be employed to condense the Mg vapors as they issue from the retort M. The most desirable procedure is to first condense the major portion of the Mg as a liquid so that it can be tapped off into molds, and to conduct the remaining vapors into a secondary condenser maintained at a temperature well below the melting point of Mg so as to condense the metal to a solid. That is to say, that it is well known that Mg vapors can not be totally condensed to a liquid, because there is appreciable vaporization in the liquid state.

In a large plant, a number of retorts such as M could discharge their Mg vapors into one large master condenser supplemented by a secondary condenser. In this way, various expedients could be adapted to afford convenience in accomplishing condensing of the Mg in two stages.

In the present instance, there is shown at W a U-tube condenser and each leg of the U-tube is connected to the pipe 130 which leads to the filter 131, a valve 129 being shown to afford alternate use of each leg. As here shown, each leg is provided with a number of heating elements such as 136. Any suitable control can be used to maintain the lower portion of the condenser at the melting point of Mg, and for this purpose it is essential that this portion be heat insulated; however, the upper part of the condenser requires no heating during condensing and therefore the upper heating elements are used only for melting down the condensed Mg. To afford efficient condensing it is advisable to provide some means for air cooling the upper part of the condenser. This air cooling may be accomplished in various ways, as for instance there is shown in Fig. 4 a casing 137 of heat insulating material vented at the top as indicated at 140 and vented at the bottom as indicated at 139 and provided with a closure sleeve 138. The bottom vents 139 are closed during the melting down of the condensed metal, after which they are opened to provide air cooling by convection. The last traces of the Mg condense as a powder, some of which passes out with the gases through the pipe 130 and is collected in the filter 131 from which the gases are returned by the pipe 132 to feed the pump 96 for recirculation through the pipes 120 and 121. Any excess gases pass through the pipe 133 into the meter N' and then through the pipe 135 to the pump 33 shown in Fig. 2.

The lower part of the condenser is provided with a pipe 141 through which the condensed magnesium is tapped off into any suitable receiver. A heating element 142 is provided to heat the pipe 141 for the purpose of tapping. For melting down the solid magnesium in the upper part of the leg, the vents 139 are closed and the

upper part of the leg heated to the required temperature, it of course being understood that the valve 129 is previously turned to close that leg and open the other.

#### Recovery of liquid hydrocarbons

As hereinbefore mentioned, the hydrocarbon vapors and gases from the separator G pass through the pipe 49 to the scrubber S. This scrubber may be of any well known type. In the present instance the scrubber S is shown with an open lower end communicating with the reservoir R which is filled with the hydrocarbon liquid which supplies the cooling spray through the pipe 28 as before explained. The liquid is maintained at a constant level by a float valve 60 which controls the flow through the pipe 25 which connects this reservoir R with the supply tank T.

As here shown the reservoir R is provided with cooling coils 56, and a motor driven pump 59 supplies a constant flow of liquid from this reservoir R to the spray ring 51 in the scrubber S for the purpose of condensing a part of the hydrocarbon vapors entering through the pipe 49. Such scrubbers are usually provided with baffles, screens or other suitable expedients, and in the present instance there is shown a number of screens 52 through which the liquid trickles to the reservoir below. Passing through the center of the scrubber is a vertical pipe 53 which connects to the center of a spiral passage 54 which has a liquid seal at the level of the liquid in the reservoir and an intake at 55 in the scrubber. Any uncondensed hydrocarbons and any gases enter this intake and are carried around the spiral passage so as to free them from suspended globules of liquid. These vapors and gases then pass through the pipe 53 and pipe 50 to the condenser C where the hydrocarbon vapors are condensed to liquid and returned to the reservoir R through the pipe 61, and the gases are passed out through the pipe 62 to the pump 33 or else are metered at N as a by-product having considerable fuel value.

As previously explained, the thermal reduction products produce sufficient blast in the flue F to satisfactorily atomize the hydrocarbon liquid sprayed into the flue through the pipe 28 and spray channel V; however, this atomization may be enhanced by recirculating the gases from the condenser C through the pump 33 and pipe 32 to the spray channel U in the flue F. In the present process, these gases contain considerably more hydrogen than carbon monoxide and there is also present some methane and minor amounts of other hydrocarbon gases; and since the shock cooling instantly dilutes these gases with several times their volume of hydrocarbon vapors, the percentage of CO is kept sufficiently low to afford satisfactory reuse of these gases without resorting to any separating of the CO. Moreover, this recirculating of these gases does not result in any accumulating percentage of CO as in other processes which do not produce hydrogen and hydrocarbon gases at the shock cooling zone. That is to say, that in the present process, the recirculated gases are the same identical gases which are produced by the process and therefore their relative percentages remain constant during repeated recirculation.

Gas analysis of the thermal decomposition of hydrocarbons occurring at the cooling zone, shows that when the shock cooling is accomplished by 75 a hydrocarbon liquid essentially non-volatile at

the shock cooling temperature employed, the amount of thermal decomposition of the hydrocarbons is minor as compared to the present process which accomplishes the shock cooling by vaporization of most of the hydrocarbon liquid. Thus the present process of shock cooling by vaporization of most of the hydrocarbon liquid, produces enough hydrogen and hydrocarbon gases to alter the percentage of CO sufficiently for satisfactory recirculation of the intermingled gases for the purpose of atomizing the hydrocarbon liquid, the vaporization of which further dilutes the CO to well within the range of successful operation.

The amount of hydrogen and hydrocarbon gases produced in the retorts L and M is not sufficient for atomizing the sprayed liquid, however, these gases which contain no CO are returned through the pipe 135 to the pump 33 and are all used for atomizing in the flue F, the additional gases necessary for the purpose being drawn into the pump 33 from the condenser C through the pipe 62, and the remainder of the flow through the pipe 62 passes through the meter N and is collected as a by-product.

#### Summary

The operation of the apparatus to perform the described process will be readily understood from the foregoing description, and it will of course be understood that the operation should be controlled so as to collect the thermal reduction products in the least amount of liquid which will afford sufficient fluidity to readily pass through the separator. It will also be understood that different liquid hydrocarbons will require a different cooling temperature to assure sufficient vaporization to leave the proper amount of unvaporized liquid for collecting, and that the amount of unvaporized liquid necessary for collecting will depend upon the amount of other solids which issue from the reduction furnace along with the Mg and CO, and that this factor will vary with different reduction furnaces or with the same reduction furnace from time to time for various reasons. It will also be understood that the temperature of the spray liquid supplied through the pipe 28 has a direct effect on the cooling temperature in the flue F and that consequently the percentage vaporization of a constant rate of flow of spray liquid will vary in accordance with the temperature of the liquid and that therefore this factor is a part of the previously described control over the percentage of vaporization.

Proper control in the various steps of the process, may be accomplished either manually or automatically, whichever mode is desired.

The molding of the briquettes in the pans of the retort F is described as the preferred practice, however, the invention can be successfully practiced by supplanting the described conveyor and pans with an endless belt of some heat resisting metal trained around pulleys. The fluid paste will readily lay on this belt and will carbonize into a porous strip, which will break into pieces of various sizes usually small, when the porous strip upon the belt starts around the pulley at the discharge end of the retort. When this practice is followed, the open ends of the cages 104 are formed with louvers or else with slots so as to more readily retain the small pieces of material, and still afford adequate passage of the circulating gas through the material in the several cages in the manner before explained.

It will of course be understood that before starting the operation of the equipment, it is necessary to displace the air in the system with some inert gas or vapor. This may be accomplished in any well known manner preliminary to the necessary preheating stage preparatory to actual operation. Once the air is displaced, the process constantly supplies an inert atmosphere of hydrocarbon vapors, hydrogen, methane, and hydrocarbon gases; and the entire system is operated under slight pressure, so as to preclude the air inleaks which might otherwise unintentionally occur with a reduced pressure within the system. That is to say, that with a slight pressure in the system, any unintended leakage will be an egress instead of an ingress; and of course any ingress of air is not only detrimental, but also dangerous because of the possibilities of explosions due to the highly combustible nature of the various substances existing in the process.

It will be readily understood that the process is directed to the commercial production of Mg from the well known MgO which has long been commercially obtained from magnesite deposits and other natural sources. The present process is readily adaptable to large scale production of Mg from MgO at a cost comparing favorably to the cost of anhydrous electrolysis of MgCl obtained from the well known magnesium bitterns or else from magnesium brines.

Where it is desired to collect the Mg and other solids in dry form, the shock cooling is accomplished by complete vaporization of a suitable hydrocarbon liquid sprayed into the flue F at the required rate. In such instances, the separator G is replaced by any suitable filter which will separate the solids from the vapors and gases, and the Mg is then recovered by distillation in any suitable manner.

The separator shown at G is made the subject of a separate application Serial No. 473,324 filed January 23, 1943; and the automatic reamer shown in Fig. 5 is made the subject of a separate application Serial No. 473,325 filed January 23, 1943.

In the present application I claim as my invention:

1. A process for producing magnesium metal, comprising thermal reduction of magnesium oxide with carbon, wherein the magnesium occurs in vapor form intermingled with carbon monoxide and some finely divided solids corresponding to the original reagents, condensing the magnesium by a spray of hydrocarbon liquid at a rate to produce a shock cooling temperature at which all of the hydrocarbon liquid is vaporized except a limited amount sufficient to form a fluid paste with the magnesium and existing solids, separating said paste from the vapors and gas, next subjecting said paste to a two stage distillation, first to distill off the hydrocarbon liquid and produce a porous solid containing finely divided magnesium, then to distill the magnesium from the porous solid, and condensing the distilled magnesium.

2. A process for producing magnesium metal, comprising thermal reduction of magnesium oxide with carbon, wherein the magnesium occurs in vapor form intermingled with carbon monoxide and some finely divided solids corresponding to the original reagents, condensing the magnesium by a spray of hydrocarbon liquid at a rate to produce a shock cooling temperature at which all of the hydrocarbon liquid is vaporized except a limited amount sufficient to form a fluid

paste with the magnesium and existing solids, separating said paste from the vapors and gas, next distilling the hydrocarbon liquid from said paste while molding the latter to form uncompressed porous cakes containing finely divided magnesium, then distilling the magnesium from the porous cakes, and condensing the distilled magnesium.

3. A process for producing magnesium metal, comprising thermal reduction of magnesium oxide with carbon, wherein the magnesium occurs in vapor form intermingled with carbon monoxide and some finely divided solids corresponding to the original reagents, condensing the magnesium by a spray of hydrocarbon liquid at a rate to produce a shock cooling temperature at which all of the hydrocarbon liquid is vaporized, removing the vapors and gas from the magnesium and other solids, and recovering the magnesium by distillation and condensing.

4. The process of producing magnesium metal, comprising thermal reduction of magnesium oxide with carbon to form magnesium vapor intermingled with carbon monoxide and some finely divided solids corresponding to the original reactants, spraying into the magnesium vapor an inert liquid at a rate to produce a shock cooling temperature by vaporization of all of said liquid except an amount which will form a fluid paste with the magnesium and other solids, separating this paste from the vaporized liquid and gas, heating the paste to vaporize the liquid from the magnesium and other solids, distilling the magnesium from the other solids and condensing the distilled magnesium, and recovering the vaporized liquid by condensation.

5. The process of producing magnesium metal, comprising thermal reduction of magnesium oxide with carbon to form magnesium vapor intermingled with carbon monoxide and some finely divided solids corresponding to the original reactants, spraying into the magnesium vapor an inert liquid at a rate to produce a shock cooling temperature by vaporization of such liquid, controlling the rate of spray so as to produce a constant temperature which will afford complete vaporization of the liquid so as to leave the magnesium and other solids in dry form, removing the vaporized liquid and gas, distilling the magnesium from the other solids and condensing the distilled magnesium, and recovering the vaporized liquid by condensation.

6. The process of producing magnesium metal which comprises, thermal reduction of magnesium oxide with carbon to produce magnesium vapor and carbon monoxide, then shock cooling the magnesium vapor to a finely divided solid metal by means of a suitable hydrocarbon liquid sprayed into the thermal reduction products at a controlled rate in direct accord with the thermal reduction output and of such ratio thereto as will produce a predetermined constant temperature within the boiling point range of the hydrocarbon liquid employed so as to be determinative of the extent of vaporization of the hydrocarbon liquid sprayed into the thermal reduction products, maintaining said predetermined constant temperature sufficiently high with relation to the boiling point range of the hydrocarbon liquid employed that the vaporization of the hydrocarbons will be sufficiently adequate to leave the magnesium in condition for immediate briquetting and recovery by distillation and condensing.

7. In a process for producing magnesium

metal wherein the magnesium occurs in vapor form in the presence of a gas and some finely divided solids, the improvement of collecting the magnesium and other solids in approximately twice their weight of a hydrocarbon liquid to thereby form a fluid paste, which comprises spraying into the magnesium vapors a suitable hydrocarbon liquid at a rate to produce shock cooling by the vaporization of all of such hydrocarbon liquid except the amount required to produce the fluid paste of aforesaid proportions, separating said paste from the vaporized hydrocarbons and gas, condensing the vaporized hydrocarbons for repeated use, distilling the unvaporized hydrocarbons from said paste to form a porous solid containing finely divided magnesium, distilling the magnesium from said porous solid, and condensing the distilled magnesium.

8. In a process for producing magnesium metal wherein the magnesium occurs in vapor form in the presence of a gas and some finely divided solids, the improvement of collecting the magnesium and other solids in approximately twice their weight of a hydrocarbon liquid to thereby form a fluid paste, which comprises spraying into the magnesium vapors a suitable hydrocarbon liquid at a rate to produce shock cooling by the vaporization of all of such hydrocarbon liquid except the amount required to produce the fluid paste of aforesaid proportions, separating said paste from the vaporized hydrocarbons and gas, condensing the vaporized hydrocarbons for repeated use, distilling the unvaporized hydrocarbons from said paste while molding the latter to form uncompressed porous cakes containing finely divided magnesium, distilling the magnesium from said porous cakes, and condensing the distilled magnesium.

9. In a process for producing magnesium metal wherein the magnesium occurs in vapor form in the presence of carbon monoxide and some finely divided solids, the improvement of collecting the magnesium and other solids in approximately twice their weight of a hydrocarbon liquid to thereby form a fluid paste, which comprises spraying into the magnesium vapors a suitable hydrocarbon liquid at a rate to produce shock cooling by the vaporization of all of such hydrocarbon liquid except the amount required to produce the fluid paste of aforesaid proportions and at the same time produce some hydrogen and methane by thermal decomposition of the hydrocarbon liquid, then separating said paste from the vaporized hydrocarbons and gases, condensing the vaporized hydrocarbons for repeated use and utilizing said gases to atomize said spray of hydrocarbon liquid, distilling most of the unvaporized hydrocarbons from said paste to form a porous solid containing finely divided magnesium and at the same time produce some hydrogen and methane by thermal decomposition of the hydrocarbons, condensing said distilled hydrocarbons for repeated use and utilizing this hydrogen and methane as a vapor carrier to accelerate distillation of said paste, distilling the magnesium from said porous solid and at the same time producing some hydrogen and methane by thermal decomposition of the existing hydrocarbon liquid, condensing the distilled magnesium, and utilizing this hydrogen and methane as a vapor carrier to accelerate distilling of the magnesium.

10. The process for producing magnesium metal, comprising thermal reduction to produce

magnesium in vapor form, condensing the magnesium vapors by direct vaporization of a spray of hydrocarbon liquid at sufficient rate to produce a shock cooling temperature which will afford a dew point to preclude vaporization of about ten per cent of the hydrocarbon liquid employed, collecting the magnesium in the unvaporized portion as a fluid paste, subjecting said paste to a two stage distillation, first to distill off the hydrocarbons and then to distill the magnesium, and condensing the latter.

11. The process for producing magnesium metal, comprising thermal reduction to produce magnesium in vapor form, condensing the magnesium vapors by direct vaporization of a spray of hydrocarbon liquid at a rate to produce a shock cooling temperature within the boiling point range of the hydrocarbon liquid employed and sufficiently below the maximum boiling point of such liquid to afford a dew point for from five to ten per cent of the liquid employed, to thereby condense the magnesium in a limited amount of hydrocarbon liquid to form a fluid paste, subjecting said paste to a two stage distillation, first to distill off the hydrocarbon liquid and then to distill the magnesium, and condensing the distilled magnesium.

12. A process for producing magnesium metal, comprising thermal reduction of magnesium oxide with carbon, wherein the magnesium occurs in vapor form intermingled with carbon monoxide and some finely divided solids corresponding to the original reactants, condensing the magnesium vapors by direct vaporization of a spray of hydrocarbon liquid at a rate to produce a shock cooling temperature within the boiling point range of the hydrocarbon liquid employed and sufficiently below the maximum boiling point of such liquid to afford a dew point for from five to ten per cent of the liquid employed, to thereby collect the magnesium and other solids in a limited amount of hydrocarbon liquid to form a fluid paste, subjecting said paste to a two stage distillation, first to distill off the hydrocarbon liquid and then to distill the magnesium, and condensing the distilled magnesium.

13. A process for condensing hot metal vapor in the presence of a reactive gas, which comprises spraying into the hot metal vapor a hydrocarbon liquid at a controlled rate in direct relation to the temperature of said metal vapor and reactive gas and of such ratio thereto as will produce a constant shock cooling temperature at which more than ninety per cent of the sprayed hydrocarbon liquid is vaporized, removing the vaporized hydrocarbons with the reactive gas and separating the latter by condensing the former, and recovering the metal by distillation and condensation.

14. A process for condensing hot metal vapor in the presence of a reactive gas, which comprises spraying into the hot metal vapor a hydrocarbon liquid at a rate to produce a shock cooling temperature by complete vaporization of the hydrocarbon liquid, removing the vaporized hydrocarbons with the reactive gas and separating the latter by condensing the former, and recovering the metal by distillation and condensation.

15. The process of producing magnesium metal, comprising thermal reduction of magnesium oxide with carbon to form magnesium vapor intermingled with carbon monoxide and some finely divided solids corresponding to the original reactants, spraying into the magnesium vapors a suitable hydrocarbon liquid at a rate to produce

shock cooling and at the same time produce an adequate amount of hydrogen and some methane by thermal decomposition of the hydrocarbons, controlling the rate of spray so that all of said hydrocarbon liquid is vaporized except an amount which will form a fluid paste with the magnesium and other solids, separating said paste from the vaporized hydrocarbons and gases, condensing the vaporized hydrocarbons for repeated use, utilizing said gases to atomize said spray of hydrocarbon liquid, distilling most of the unvaporized hydrocarbons from said paste to form a porous solid containing finely divided magnesium and at the same time produce some hydrogen and methane by thermal decomposition of the hydrocarbons, condensing said distilled hydrocarbons for repeated use and utilizing this hydrogen and methane as a vapor carrier to accelerate distillation of said paste, distilling the magnesium from said porous solid and at the same time producing some hydrogen and methane by thermal decomposition of the existing hydrocarbon liquid, condensing the distilled magnesium, and utilizing this hydrogen and methane as a vapor carrier to accelerate distilling of the magnesium.

16. The process of producing magnesium metal, comprising thermal reduction of magnesium oxide with carbon to form magnesium vapor intermingled with carbon monoxide and some finely divided solids corresponding to the original reactants, spraying into the magnesium vapors a suitable hydrocarbon liquid at a rate to produce shock cooling and at the same time produce an adequate amount of hydrogen and some methane by thermal decomposition of the hydrocarbons, controlling the rate of spray so that all of said hydrocarbon liquid is vaporized except an amount which will form a fluid paste with the magnesium and other solids, separating said paste from the vaporized hydrocarbons and gases, condensing the vaporized hydrocarbons for repeated use, utilizing said gases to atomize said spray of hydrocarbon liquid, distilling the unvaporized hydrocarbons from said paste to form a porous solid containing finely divided magnesium, distilling the magnesium from said porous solid, and condensing the distilled magnesium.

17. The process of producing magnesium metal, comprising thermal reduction of magnesium oxide with carbon to form magnesium vapor intermingled with carbon monoxide and some finely divided solids corresponding to the original reactants, spraying into the magnesium vapor a suitable hydrocarbon liquid at a rate to produce shock cooling and at the same time produce an adequate amount of hydrogen and some methane by thermal decomposition of the hydrocarbons, controlling the rate of spray so as to vaporize all of said hydrocarbon liquid and leave the magnesium and other solids in dry form, removing the vaporized hydrocarbons and said gases, separating the latter by condensing the former, utilizing said gases to atomize said spray of hydrocarbon liquid, and separating the magnesium from the other solids by distillation and condensing.

18. A process for condensing hot metal vapor in the presence of a reactive gas, which comprises spraying into the hot metal vapor a suitable hydrocarbon liquid at a rate to produce shock cooling and at the same time produce an adequate amount of hydrogen and some methane by thermal decomposition of the hydrocarbons, controlling the rate of spray so as to vaporize all of said hydrocarbon liquid, removing the vaporized hy-

drocarbons and said gases, separating the latter by condensing the former, and utilizing said gases to atomize said spray of hydrocarbon liquid.

19. In a process for producing magnesium metal by thermal reduction of magnesium oxide with carbon to produce magnesium vapor and carbon monoxide, the step which comprises shock cooling the magnesium vapor to a finely divided solid metal by means of a suitable hydrocarbon

liquid sprayed into the thermal reduction products at a controlled rate so as to produce a predetermined temperature at which the vaporization of the hydrocarbons will be sufficiently adequate to leave the magnesium in condition for immediate briquetting and recovery by distillation and condensing.

HENRY A. DOERNER.

CERTIFICATE OF CORRECTION.

Patent No. 2,328,202.

August 31, 1943.

HENRY A. DOERNER.

It is hereby certified that error appears in the printed specification of the above numbered patent requiring correction as follows: Page 1, first column, line 18, for "fluid" read --flue--; page 10, first column, line 13, claim 11, for "ocmpri sing" read --comprising--; and that the said Letters Patent should be read with this correction therein that the same may conform to the record of the case in the Patent Office.

Signed and sealed this 30th day of November, A. D. 1943.

(Seal)

Henry Van Arsdale,  
Acting Commissioner of Patents.